

# UNITED STATES PATENT OFFICE.

JAMES F. O'BRIEN, OF CHICAGO, ILLINOIS.

## EXPLOSIVE.

1,071,949.

Specification of Letters Patent.

Patented Sept. 2, 1913.

No Drawing.

Application filed September 16, 1912. Serial No. 720,458.

To all whom it may concern:

Be it known that I, JAMES F. O'BRIEN, a citizen of the United States, residing at Chicago, in the county of Cook, State of Illinois, have invented new and useful Improvements in Explosives, of which the following is a specification.

This invention relates to improvements in my potassium chlorate explosives and particularly to improvements in my potassium chlorate hydro-carbonaceous explosive set forth in my application filed June 3, 1912, bearing S. N. 701,258; and the improvement to be particularly dealt with in this application consists in a waterproof explosive made wholly (or essentially wholly) of a chlorate, a hydro-carbonaceous material or materials and a silicious material or materials. In a co-pending application filed September 16, 1912, Ser. No. 720,459 I have explained another explosive consisting exclusively of chlorate and hydro-carbonaceous materials; and this and the present explosive have practically the same objects.

There are many objects of the present invention; and I may mention the following as being some of the most important: first, the reduction in cost and increase in safety of manufacture without a reduction in explosive efficiency; second, the use of common and inexpensive materials in the manufacture of the explosive; third, the manufacture of the complete explosive ready for package by one simple operation; fourth, the practical non-delicquescence of the final product (this is an important feature as it means non-deterioration in presence of water and consequent safety); fifth, the elimination of carbo-hydrates—comparatively expensive—the substitution of hydro-carbonaceous materials—comparatively inexpensive; sixth, elimination of tackiness or stickiness, thus avoiding dangerous friction both in mixing and use; and seventh, the final provision of an explosive suitably plastic for handling in cartridge form, and water-proof in itself. The last object is the primary and most important one of this carbonaceous material explosive; and it is of very great importance that the explosive is water-proof in itself—by virtue of its essential ingredients—and needs no external or other application to render it proof against moisture. The elimination of the carbo-hydrates, above noted, has several advantages, which may also be considered objects

of my invention. In the first place, hydrocarbons are generally cheaper than carbohydrates; the hydro-carbons make for higher temperature and greater gas volume—therefore greater explosive energy; and the hydro-carbon explosive is safer to handle on account of its lesser susceptibility to jar, vibration or shock.

In my application Ser. No. 701,258, filed June 3, 1912, I have set forth an explosive which contains a chlorate, a carbo-hydrate, a carbonaceous material and silicious material. In my present explosive I employ only chlorate, carbonaceous materials and silicious material as the base or fundamental of my explosive; I may add other ingredients, such as powdered charcoal or stone coal, and ferro-cyanid of potassium, but these ingredients and others of similar nature which may be added, are of not as vital importance to the explosive as the fundamental and basic ingredients.

I have exhaustively experimented with the combination herein set forth and I have found that I am enabled to obtain excellent results with a combination of a chlorate, one or more of many forms of hydro-carbons, and one or more of the many forms of silicious materials. Generally speaking, I have found that silicious materials containing silicon and oxygen in combination are suitable for my explosive; and I may prefer to use silica on account of its availability and cheapness. The matter of choice of particular hydro-carbons has largely been influenced by questions of manufacture. As finally selected (as indicated in the following formulæ) the hydro-carbons lend themselves largely to ease in manufacture of the explosive in a single simple mixing operation; and it is these hydro-carbons which, in connection with the other ingredients, make the whole composition water-proof in itself. By suitably selecting the hydro-carbons I eliminate entirely the necessity of granulating, drying, insulating and water proofing preparatory to use; it only becomes necessary to pack the plastic product into a suitable cartridge, when it is ready for shipment and use, as will be hereinafter explained.

I will now herewith give a typical formula for my explosive and will explain in detail the manufacture; I will then give a modified formula, adding some ingredients. And I will also explain the particular rea-

sons for selecting the particular hydro-carbons set forth, explaining generally how other hydro-carbons could be substituted for those chosen and still have the same reaction 5 and more or less closely the same explosive efficiency.

The basis or fundamental of my explosive is preferably composed as follows:

|    |                    |            |
|----|--------------------|------------|
| 10 | Potassium chlorate | 87.0 parts |
|    | Naphthalene        | 6.5 "      |
|    | Asphalt            | 6.5 "      |
|    | Distillate         | 1.5 "      |
|    | Silicious material | 44.0 "     |

15 I may vary this formula by adding to it a small amount of powdered stone coal or charcoal and a small amount of ferro-cyanid of potassium, so the formula reads as follows:

|    |                                 |            |
|----|---------------------------------|------------|
| 20 | Potassium chlorate              | 87.0 parts |
|    | Naphthalene                     | 6.5 "      |
|    | Asphalt                         | 6.5 "      |
|    | Distillate                      | 1.5 "      |
|    | Silicious material              | 44.0 "     |
| 25 | Powdered stone coal or charcoal | 2.0 "      |
|    | Ferro-cyanid of potassium       | 1.0 "      |

In the process of manufacture of this preferred form of my explosive, I first dissolve the asphalt and naphthalene in just sufficient distillate (ordinary engine distillate from asphalt base and of 50-51 Baumé gravity being generally used) to make the whole solution flow well. The quantity of 30 distillate necessary for this solution may vary somewhat; but I have given a general fair average in the above tabulation. The asphalt is preferably provided in a crude oil product generally known as "road oil", 35 which is the residue of crude oil after refining treatment to approximately 700 degrees F. The road oil used by me in my explosive has generally contained ninety per cent. asphalt and ten per cent. other hydro-carbon liquids; and, when the asphalt is 40 used in this form, the whole volume of road oil is mixed with the naphthalene and distillate to form a smoothly flowing fluid. The naphthalene used is preferably in the form 45 of "naphthalene salts", which is the impure, coarsely crystalline article of commerce known otherwise as crude naphthalene. The fluid is then in condition to mix well and thoroughly with the solid ingredients. The solid ingredients (the chlorate and 50 silicious materials) are then mixed together; and then the prepared liquid is mixed with the prepared solids in a single, special mixing machine which is frictionless and non-confined. In this connection I may again 55 mention the smooth, frictionless qualities of my explosive; the mass will not create friction in a machine as it slides smoothly over and around the mixing drum and fingers. 60 The amount of liquid in the prepared fluid

is just sufficient to give to the final product a plasticity which renders the final product easily handled and easily packed into cartridges. The final product is of somewhat the consistency of cheese, being easily cut and easily pressed into any shape. The silicious material preferred by me is ordinary silica; but I have found equivalents which give much the same action as silica, such an equivalent being powdered brick 70 dust, a silico-aluminous material. 75

Hydro-carbons other than those above set forth may be used in my combination without materially changing the essentials of the explosive combination; but the above 80 described combination has not only the advantage of great explosive energy and efficiency, but also has the advantage of mixing simply to form a final, practically water-proof product of the desired consistency. I have selected the combination above set forth first with regard to water-proof qualities of the final product, and then largely on the grounds of simplicity of manufacture, and largely on the ground of 85 cheapness. (Provided always that the efficiency of the explosive is not lessened.) Each of the selected ingredients is readily obtainable in sufficient quantities to be entirely practicable of use for the large manufacture of an explosive. 90

I may use a small amount of powdered stone coal or charcoal for the process of transmitting flame throughout the finished stick or cartridge of the explosive. This 100 powdered carbon is thoroughly mixed with the other ingredients so that it is uniformly distributed and will carry flame throughout the mass. The ferrocyanid of potassium may be added to change the speed of the 105 detonation.

This form of explosive has all of the advantages of the explosives heretofore set forth by me, and has in addition the very important advantage of being cheap and 110 simple of manufacture. It is seen from the foregoing description that not only are the ingredients cheap and universally obtainable, but also the method of manufacture is extremely simple, requiring only a single 115 mixing operation in a simple machine. When the explosive is finished it has a smooth water repelling surface; there is no stickiness or tackiness, and the mass of explosive is practically water-proof. The 120 mass is essentially homogeneous throughout and uniformly plastic. It may be formed into any desired shape and may be cut very easily. It is non-deliquescent, the small deliquescence of the chlorate being "bound 125 in" by the practically water-proof plastic mixture. The chlorate is the only substance in the powder which has any tendency whatever to take up water; the other substances are water-proof in themselves. 130

These water-proof substances are sufficient to entirely bind in the chlorate; and thus make a composition almost water-proof in itself. Being practically water-proof, it will not deteriorate in presence of moisture; this means that the original strength and safety of the explosive are maintained unimpaired. These features are of highest importance. The labor of packaging this new explosive is very slight as compared with others; its plasticity makes it easily formed into cartridges and sticks. In manufacture, actual use and in transportation it is remarkably safe to handle; a stick has been fired into with a United States Army rifle of thirty caliber without any effect whatever. A double strength electric cap has caused ignition but not explosion. When ignited openly it burns rapidly but does not detonate. It is chemically stable under all ordinary temperatures and safe for transportation within all reasonable and ordinary limits. In energy of explosion it is classed as a high explosive, giving results comparable with the highest grade of commercial dynamite. When placed in a hole it may be tamped indifferently without any fear of detonation; it has no sensibility to shock or percussion. It is not necessary to use a cap in detonating this explosive; an ordinary fuse will cause complete and unfailing explosion when the explosive is confined, causing only rapid combustion when unconfined.

In the following claims I seek to secure to myself those combinations which make a practically water-proof safe explosive manufactured in a simple and safe manner in a single operation; producing an explo-

sive practically water-proof in itself, of great explosive energy, safe to handle, non-deteriorating and capable of detonation by a common fuse when ignited.

Having described my invention, I claim:

1. An explosive, comprising potassium chlorate, asphalt, crude oil distillate, and silica. 45

2. An explosive, comprising potassium chlorate, naphthalene and asphalt dissolved in crude oil distillate, and silica. 50

3. An explosive, comprising potassium chlorate, naphthalene and asphalt dissolved in crude oil distillate, carbon in powdered form, and silica.

4. An explosive, comprising potassium chlorate, naphthalene and asphalt dissolved in crude oil distillate, powdered carbon, ferro-cyanid of potassium, and silica. 55

5. An explosive, comprising approximately potassium chlorate eighty seven 60 parts, naphthalene six and one half parts, asphalt six and one half parts, crude oil distillate one and one half parts, and silica forty four parts.

6. An explosive, comprising approximately potassium chlorate eighty seven 65 parts, naphthalene six and one half parts, asphalt six and one half parts, crude oil distillate one and one half parts, powdered carbon two parts, ferro-cyanid of potassium 70 one part, and silica forty four parts.

In witness that I claim the foregoing I have hereunto subscribed my name this 9th day of September 1912.

JAMES F. O'BRIEN.

Witnesses:

ELWOOD H. BARKELEW,

W. L. CONNOR.

Copies of this patent may be obtained for five cents each, by addressing the "Commissioner of Patents, Washington, D. C."